

H. L. CHARLES.

REVERBERATORY FURNACE.

APPLICATION FILED AUG. 30, 1917. RENEWED JAN. 23, 1920.

1,351,835.

Patented Sept. 7, 1920.

2 SHEETS—SHEET 1.



INVENTOR

Henry L. Charles.

BY  
*Thos. A. Hill.*  
ATTORNEY

1,351,835.

H. L. CHARLES.

REVERBERATORY FURNACE.

APPLICATION FILED AUG. 30, 1917. RENEWED JAN. 23, 1920.

Patented Sept. 7, 1920.

2 SHEETS—SHEET 2.



# UNITED STATES PATENT OFFICE.

HENRY L. CHARLES, OF BUTTE, MONTANA.

## REVERBERATORY FURNACE.

1,351,835.

Specification of Letters Patent. Patented Sept. 7, 1920.

Application filed August 30, 1917, Serial No. 188,889. Renewed January 23, 1920. Serial No. 353,589.

To all whom it may concern:

Be it known that I, HENRY L. CHARLES, a citizen of the United States, residing at Butte, in the county of Silver Bow and State of Montana, have invented certain new and useful Improvements in Reverberatory Furnaces, of which the following is a specification, reference being had therein to the accompanying drawing.

10 My invention relates to improvements in the method of feeding reverberatory smelting furnaces, and is in the nature of an improvement upon my United States Patent No. 871,477, granted November 19, 1907. 15 In my previous patent, I disclosed the method of feeding the raw silicious ores against the side walls of the furnace to prevent the molten slag, matte or any of the sulfids from touching the brick lining, corroding the wall around the hearth, instead of charging the furnace so as to cover the hearth several inches deep, leaving the walls exposed to corrosion.

According to my present method of feeding the furnace, I prefer to feed the metallic ores such as copper, iron, nickel, zinc, etc., calcines, flue-dust, silicious ores, copper chips, slag, copper or iron refuse in rows or a series of mounds or piles from hoppers 25 above the roof, so that the ores to be smelted will pile upon the hearth, presenting a much larger surface exposed to the heat. By this method, when ore is brought to a point at the top of a pile or mound to be smelted, it 30 will frit down the sides of the pile or mound much master than when the ore is lying substantially flat upon the hearth, and as soon as the melted ore flows away, it leaves fresh ore exposed to the heat, whereas 35 in present practice, the ore remains blanketed over the center of the hearth, making it difficult for the heat to penetrate and melt the ore beneath. It may also be desirable to have the rear mounds or piles of ore 40 higher than the piles or mounds at the center and at the front end of the hearth thereby producing the effect of a gradual slope of ore mounds toward the front ends of the furnace, and I prefer that the bottom 45 of the hearth be given a slight slope toward the front, and that the front of the hearth be much deeper than usual to act as a receiver for the molten metal and slag. Fluxes of any suitable kind can also be fed 50 if desirable to clean the slag. Copper scraps, iron scraps or ores may also be fed,

and I have found that the grade of matte can be raised or lowered when properly handled at this point.

Referring to the accompanying drawings, 60 I have illustrated in Figure 1, partly in longitudinal cross section, the usual form of reverberatory furnace, illustrating an embodiment of my invention. Fig. 2 is a plan view of the line 2—2 of Fig. 1. Fig. 65 3, a cross sectional view of such a furnace on the line 3—3 of Fig. 1, and Figs. 4 and 5 also cross sectional views of such a furnace on the lines 4—4 and 5—5 respectively of Fig. 1. 6 indicates the usual furnace 70 foundation, and 7 the bed of the furnace, provided with a bridge wall such as 8, at one side of which is provided the grate bars 9, from which the flame and gases from the fire pass rightwardly over the brick wall 75 along the entire furnace escaping at the right, or front end of the furnace through the usual flue not shown.

9'—10—11 indicate the piles or mounds of metallic ores to be smelted, and the piles 80 or mounds are formed by the ores dropping from the hoppers 12—13—14 immediately above.

I have found that to feed coarse or lumps of ore, slag or copper chips first upon the 85 hearth, and the finer ores last, such as flue-dust, calcine concentrates, slimes, etc., raw or roasted, that it is easier to maintain the piles or mounds in shape. The finer products, such as flue-dust, calcines, ores etc., 90 will if hot, spread over a large area faster in a molten bath of metal and slag, than if they are fed upon a dry hearth, however, I do not of course limit myself to either method of proceeding, and the piles or 95 mounds may be maintained after the smelting has begun, and any furnace in operation can be used in the application of my method, while the furnace is at full heat, 100 and while full of molten metal and slag.

In the construction of a furnace, it may be desirable to build these mounds of any suitable refractory material, so as to maintain the continuous shape of the mound, although it may of course be found preferable to form the mounds or piles of a 105 fusible ore.

As the flame and gases pass rightwardly, looking at Fig. 1 at the front of the furnace, the pointed peaks of the mounds or piles 110 such as indicated by the reference character 10, round off and drop down, leaving the

piles or mounds more rounded and reduced at the top as indicated by the reference character 9', and for the purpose of restoring the peaks or points of the mounds, additional ore may be discharged from the proper hoppers immediately upon the mounds as required, and while the smelting operation is going on.

While I have shown in Fig. 2 a staggered arrangement and means at the left of said figure, it may of course in some instances be desirable to arrange the mounds in a row or rows, such as illustrated at the right of Fig. 2 in dotted outline, and I also of course prefer to mound the ore against the wall of the furnace as shown, and as specified in my previous patent referred to.

The last mounds indicated by the reference character 11 in Fig. 1, I may prefer to maintain in reduced size as shown, thus facilitating the accumulation of the matte 12 and slag 13 at the front of the furnace.

From the foregoing, it will be readily understood that a very much larger surface 25 of ore is thus presented to the intensely hot gases and flame of the furnace and that as the finer ore upon the top and sides of the mounds or piles is melted and run off, additional ore may be constantly supplied thereon by maintaining a large surface presented to the heat of the furnace, thus hastening the smelting operation and providing an arrangement practically automatic for continuous operation. By staggering the piles 30 or mounds of ore as shown at the left of Fig. 2 the flame and furnace gases are obliged to lick around the mounds thoroughly contacting through whereas in the old practice the larger portion of these hot 35 gases passed right through the furnace without contacting with the ores. It will also be found that by first charging the hoppers with the coarser ores and subsequently with

more finely divided ores and still finer as the top of the mounds or piles are approached 45 until finally depositing a mere dust that a quicker and more efficient working will be provided and as the mounds settle, it is preferable to first add some of the coarser ore upon the top of the settled mound before 50 adding the finer ore to form the peaks.

Of course it will be understood that various modifications may be made in the construction and arrangement of parts and in the several steps of my invention without departing from the spirit of the invention 55 as claimed.

I claim:

1. The within described method of feeding ores into a reverberatory furnace consisting in dropping the same upon the hearth in such a manner as to provide piles 60 or mounds at frequent intervals.

2. The within described method of feeding ores into a reverberatory furnace which 65 consists in dropping the same upon the hearth in such a manner as to provide piles or mounds at frequent intervals, and at pre-determined places.

3. The within described method of feeding ores into a reverberatory furnace consisting in dropping the ores upon the hearth in small piles at short intervals whereby a maximum surface of the ores is presented. 70

4. The within described method of feeding ores into a reverberatory furnace consisting in discharging the same upon the hearth by first feeding the coarser portions 75 of the ore, then the finer portions thereafter.

In testimony whereof I hereunto affix my 8 signature in the presence of two witnesses.

HENRY L. CHARLES.

Witnesses:

ETHEL G. GARDNER,  
ANNA F. DUFFY.